

## UNITED STATES PATENT OFFICE.

ERNEST S. FISHER, OF SALT LAKE CITY, UTAH, ASSIGNOR TO UTAH METALS FLUX COMPANY, OF SALT LAKE CITY, UTAH, A CORPORATION OF UTAH.

## METHOD OF IMPROVING FERROUS METALS AND PRODUCTS THEREOF.

No Drawing. Original application filed June 25, 1924, Serial No. 722,409. Divided and this application filed August 20, 1926. Serial No. 130,561.

This invention relates to methods of improving ferrous metals, and particularly to treatments in which substances are either added for this purpose to a fused bath of the 5 metal or applied to the solid metal while at a substantially elevated temperature.

More particularly my invention relates to the improving of ferrous metals by the action of certain naturally occurring deposits which 10 have been found to not only purify the metals but positively to impart to the same desirable mechanical characteristics.

I have found that there are certain deposits of shale which possess the property of effecting the improvements mentioned. One such deposit is in the northern-central portion of Emery County, Utah, south of the Price River and Desert Lake. This shale, which is to be distinguished from the blue or blue-gray variety found in the same vicinity, is a highly laminated carbonaceous or bituminous shale varying in color from dark brown or almost black through brown to brick-red, with frequently a yellowish tint on the 20 surfaces of the laminae.

The shale is susceptible of quite varied use in metallurgical operations, but I shall confine the present description mainly to certain of the uses which have been thoroughly tried 30 out and the products of which have proved thoroughly satisfactory.

If from 1 to 10 percent by weight of this shale is cooked with scrap iron, even poor grades of cast iron, there results from the 35 melt a product which is clean, solid, and malleable and the tensile strength of which is enormously increased. Castings made directly from the bath are clean, more free from fins than cast iron castings, and readily workable, and may be machined at much higher 40 speed than customarily can be employed in working cast iron. Castings of this product may be made much lighter than heretofore on account of the strength of the product and 45 its highly dense and fibrous nature.

Iron treated according to my method may be welded without the use of a flux, and in this manner distinguishes greatly from cast iron. Using sticks or the like made of the 50 treated iron as welding rods enables cast iron pieces to be welded together without the use of other fluxing media. In either case the welds are not hardened and are as machinable

as the original pieces. On many tests, the welds proved stronger than the original 55 pieces.

I find in general that an addition of from 1 to about 6 percent of the shale to the molten bath softens and toughens the product, while higher proportions of the shale have a hardening effect.

Another useful application of my invention is in cupola practice. I have found that the addition of from 1 to 15 percent by weight of the shale to the charge of iron or iron-containing metals and coke or other fuel in the cupola furnace not only produces the improvements and characteristics referred to, in the batch to which the shale has been directly added, but that the effect of the flux 70 or agent permeates the superincumbent charges to an appreciable extent; so much so that the foundrymen will recognize the product at once on casting and machining. The vapors evolved in the heating process therefore carry to some extent the active substance of the shale, although of course the effect is most noticeable in the molten portion of the charge to which the flux has been directly added. The cupola treatment softens the 80 texture, fiber or grain of the metal, toughens the same and strengthens the casting, producing in effect a casting similar to a wrought or malleable iron; at the same time practically eliminating and freeing the same from 85 any oxygen, nitrogen or other deleterious elements, thus producing a solid, sound casting free from blow-holes or other imperfections.

Relative to the extent to which the treatment described improves the metal, I may 90 state that the average transverse strength of good cast iron is in the neighborhood of from 2500 to 2900 pounds, whereas castings of iron made in accordance herewith test from 3600 to 4500 pounds per square inch transverse 95 strength.

The improvements noted as to treated cast iron are equally obtained in the treatment of steel.

Molten cast iron when contacted with from 100 four to six percent of the shale as heretofore described when used in welding cast iron to cast iron produces, without the use of any other flux, a joint which is exceptionally strong and easily machined and which is 105 practically free from pittings or gas holes.

I do not know at the present time exactly what the effect is due to, but I believe that it results from a complex reaction between certain of the constituents of the shale and of the metals, and possibly the isolation of some unknown material which acts, perhaps catalytically, to homogenize and condense the metal in its presence.

An average analysis of this shale shows its composition to be about as follows:

|                    |              |
|--------------------|--------------|
| 15 Silica          | 45%          |
| Iron oxide         | 10%          |
| Aluminum oxide     | 12%          |
| Calcium oxide      | 2.5%         |
| 15 Magnesium oxide | 1%           |
| Sulphur            | .087%        |
| Phosphorus         | .068%        |
| Alkalies           | 1.81%        |
| 20 Titanium        | Trace        |
| Vanadium           | .013 - 5%    |
| Uranium            | Trace - .37% |
| Carbon             | 10.24%       |

It is to be understood that the titanium, vanadium and uranium components of the said shale occur not as free elements but in the form of compounds,—probably as oxides, carbides or sulfides,—thereof.

It is possible that other samples of this shale capable of effecting the results mentioned will vary considerably in proportions in the majority of ingredients mentioned, but the above is an average analysis of the particular shale in the region described.

35 The various analyses which have been made show losses on ignition varying from 15 to 31 percent. It is possible that some of the substances thus lost on ignition play an important part in the mechanism of the reaction which occurs. This theory is borne out in part by the fact that the upper layers of the charge in a cupola or similar furnace undergo improvement which is quite noticeable, although the shale itself is added and 40 confined to the lowermost portion of the charge.

Of course the slag which is formed upon melting is removed before or upon pouring.

50 Metals, particularly impure scrap iron, when treated as described, lose weight to some extent, probably due to the scavenging action of the shale.

It will be understood where I have stated in the appended claims that the shale is introduced into the molten bath, I also contemplate the introduction of the shale into the

crucible, furnace or other apparatus either before, along with or subsequent to the introduction of the metal or metals.

This application is a division of my co-pending application Serial No. 722,409, filed June 25, 1924.

I claim:

1. Method of improving ferrous metals which comprises contacting the same in molten state with a composition substantially identical with the carbonaceous shale found in the northern central portion of Emery County, Utah, south of Price River and Desert Lake.

2. Method of improving iron which comprises contacting the same in molten state with a composition substantially identical with the carbonaceous shale found in the northern central portion of Emery County, Utah, south of Price River and Desert Lake.

3. Method of producing malleable cast iron having physical characteristics of wrought iron which comprises melting cast iron and introducing thereinto about from 1 to 15% by weight of a composition substantially identical with the carbonaceous shale found in the northern central portion of Emery County, Utah, south of Price River and Desert Lake, and casting the metal into shape in suitable molds.

4. Method of improving steel which comprises contacting the same in molten state with a composition substantially identical with the carbonaceous shale found in the northern central portion of Emery County, Utah, south of Price River and Desert Lake.

5. Malleable cast iron possessing the physical characteristics of wrought iron, produced by subjecting molten cast iron to the influence of a heated composition substantially identical with the carbonaceous shale found in the northern central portion of Emery County, Utah, south of Price River and Desert Lake.

6. Method of producing iron for welding rods which comprises establishing a molten bath of cast iron and introducing thereinto from 4 to 6 percent by weight of a composition substantially identical with the carbonaceous shale found in the northern central portion of Emery County, Utah, south of Price River and Desert Lake, and forming the metal into rods.

In testimony whereof, I affix my signature.

ERNEST S. FISHER.